

E. RICHARDSON.

TABLE.

APPLICATION FILED MAR. 9, 1915.

1,161,975.

Patented Nov. 30, 1915.

*Fig. 1.*



*Fig. 2.*



*Fig. 3.*



WITNESSES

R. F. Dilworth  
Elva Stanick

INVENTOR

Ernest Richardson  
by G. N. Barber  
attorney

# UNITED STATES PATENT OFFICE.

ERNEST RICHARDSON, OF COLLEGE HILL, PENNSYLVANIA.

## TABLE.

1,161,975.

Specification of Letters Patent. Patented Nov. 30, 1915.

Application filed March 9, 1915. Serial No. 13,138.

*To all whom it may concern:*

Be it known that I, ERNEST RICHARDSON, a citizen of the United States, residing at College Hill, in the county of Beaver and 5 State of Pennsylvania, have invented new and useful Improvements in Tables, of which the following is a specification.

My invention relates to tables or similar articles having porcelain enameled metal 10 tops.

It is one of the objects of this invention to construct the sheet metal for table tops, kitchen cabinet tops, and the like so that they will not warp or buckle in the enamel 15 burning furnace or during their cooling after having been removed therefrom.

Another object is to manufacture the said tops with enameled border flanges so that the enamel on the flanges will not be cracked 20 or broken by reason of blows thereon received during the shipment of the tops or during their subsequent use. My table tops are extensively used in restaurants in which the tables are pushed about carelessly, par- 25 ticularly while the floors are being cleaned, whereby the corners of some of the tables strike the flanged sides of other tables and crack or break the enamel thereon when the enamel is applied to the flanges in the usual 30 manner or in the same manner in which it is applied to the upper surface of the tops.

Another object is to provide the enamel on the said flanges with a color coat applied in flecks or small spots in order to prevent 35 the color coat from chipping off or cracking as a color coat is liable to do when it receives hard blows or extreme changes in temperature.

A still further object of my invention is 40 to secure the said tops to a table cabinet or other body or support in a convenient and cheap manner.

Referring to the accompanying drawings, Figure 1 is a perspective of a table embodying the principles of my invention, the lower portions of the legs being broken away; Fig. 2 is a section of Fig. 1 on the line II—II; and Fig. 3 is a bottom plan view of the table one side being broken 50 away.

The table top 1 comprises a thin layer of metal, preferably pressed sheet metal 2, coated with porcelain enamel. The sheet metal 2, which is initially flat, has its central portion 3 depressed slightly so as to leave a narrow border 4 extending entirely

around the top 1. This border is comparatively narrow and serves, with the flange 5 depending from the edges of the top 1, to stiffen the metal so that it will not warp or buckle during the time the top is in the enamel burning furnace or while it is cooling after it has been taken therefrom. It was found that the said flange alone would not prevent the metal from warping or twisting out of shape, but that by depressing the metal from near the edges of the top 1 the latter would remain in its normal flat condition during and after its treatment in the said furnace.

After the sheet metal 2 has been given the depression 3 and the border 4 and provided with the border flange 5, I coat the top with the coat 6 of enamel which I have shown on the upper side of the top and on the outer face of the flange 5, though it may cover the remaining surface of the top, if desired. This coat of enamel is preferably without porcelain enamel coloring matter and is very thin. It may be clear enamel applied in such a thin layer as to show the dark surface of the metal through it, as shown by the dark ground color on the flange 5 (Fig. 1). The layer 6 of enamel must be so thin on the flange 5 that it will not chip off or crack when subjected to hard blows, or rapid or extreme changes of temperature. The coated metal top is subjected to the action of a suitable enamel burning furnace in which the enamel is fused on the metal. After the 75 coated metal has been taken from the furnace and allowed to cool, the coat 6 is covered with the color coat of enamel, which is spread in an even layer 7 over the upper surface of the top but is applied in flecks or spots 8 of small area on the coat 6 on the flange 5. It has been found that the flecks 8 will not chip off or crack when subjected to very hard blows or to sudden or extreme changes of temperature.

The coloring material in the second coat renders it somewhat brittle, and requires it to be considerably thicker than uncolored coats are required to be. Consequently, the first, or ground, coat 6 being without color (or at 90 least having a very little coloring matter) may be very thin, and the second coat, containing color may be thick on the flange 5 provided it be in spots or flecks of small area. The spots or flecks can freely expand 95 edgewise without danger of their breaking or cracking, and the smallness of the spots

or flecks prevent their chipping or cracking, this result being secured in part at least by the fact that the enamel in the spots or flecks becomes gradually thinner toward their edges.

- The table body comprises a rectangular frame composed of strips 9 of sheet metal arranged at right angles to the top 1 and within the area bordered by the flange 5.
- 10 The strips 9 are bolted or riveted to the metal legs 10 which are V-shaped in cross-section. Wooden strips 11 lie between opposite strips 9 with the ends of the former abutting against the inner faces of the said strips 9. Screws 12 extend through the flange 5 into the ends of the wooden strips and secure the top 1 to the wooden strips. The metal strips 9 have lugs or ears 13 bent at right angles thereto, on which the said 20 wooden strips 11 rest. The ears 13 and the strips 11 are secured together by the bolts 14 and nuts 15.

This application is a continuation in part of my application Serial Number 829,002, filed April 2, 1914.

I claim—

1. In a table or the like, a sheet-metal top having a depending flange on the edges thereof, a coat of enamel on the upper sur-

face of the top, the said enamel containing 30 porcelain enamel coloring material, a coat of enamel on the exterior surface of the flange, the latter enamel being substantially free from said coloring material and so thin as to prevent its breaking or cracking when subjected to severe blows, and flecks of enamel containing said coloring matter on the 35 said enamel on the flange.

2. In a table or the like, a sheet-metal top having a depending flange on the edges 40 thereof, a coat of enamel on the exterior surface of the flange, the said coat being so thin as to prevent its breaking or cracking when subjected to severe blows, and flecks of enamel containing coloring matter on the 45 said thin enamel.

3. In a table or the like, a sheet-metal top having a depending flange on the edges thereof, a coat of enamel on the exterior surface of the flange, and flecks of enamel containing 50 coloring matter on the said enamel.

Signel at Beaver Falls, this 4th day of March, A. D. 1915.

ERNEST RICHARDSON.

Witnesses:

H. F. HAWKINS,  
LOUIS MEPEAU.